# EUROPEAN PATENT APPLICATION

(11) **EP 0 011 488 A1**
(43) Date of publication of application: **28.05.1980**
(21) Application number: 79302579.2
(22) Date of filing: 14.11.1979
(51) Int. Cl.: D21H 5/00, C08J 5/00

(54) **Heat bonded paper**

(30) Priority: 17.11.1978 GB 7844903
(71) Applicant: The Wiggins Teape Group Limited, Basingstoke Hampshire RG21 2EE (GB)
(72) Inventor: Drew, Quentin Miles, Tiverton Devon (GB); Nicholas, Roger Philip, Cullompton Devon (GB)
(74) Representative: Carmichael, David Andrew Halliday

(57) **Abstract**

This invention relates to a heat bonded paper web comprising cellulosic fibres, synthetic thermoplastic fibres and a resinous additive. It has been found that the tear strength, tensile strength and stretch properties of the heat bonded web are improved by adding a resinous additive to the paper before heat bonding. Paper according to the invention is particularly suitable for base paper for book binding.

## Description

This invention relates to heat-bonded paper webs made from a blend of natural cellulosic fibres and'synthetic thermoplastic fibres.

Paper webs have traditionally been formed from cellulosic fibres derived from various materials of vegetable origin, for example woodpulp. Where it is desirable for the web to be susceptible to heat treatment, it has been proposed to incorporate a proportion of synthetic thermoplastic fibres in the web. Originally, chopped staple fibres were proposed for this purpose. However, such fibres are unfibrillated and incapable of hydrogen bonding, and thus they are inherently unsuited to the production of strong paper webs. With the exception of one or two speciality products therefore, the inclusion of chopped staple fibres in paper webs has not been widespread.

In recent years, so-called synthetic woodpulp fibres have become available. These fibres are produced specially for use in papermaking, and have a gross morphology (i.e. length: diameter ratio) and diameter of the same order-of magnitude as cellulosic papermaking fibres derived from woodpulp. They also resemble cellulosic fibres in being fibrillated to a considerable extent, and they thus permit stronger webs to be obtained than is the case with chopped staple fibres. Examples of commercially-available synthetic wood- pulps are "SWP" supplied by Crown Zellerbach, "Pulpex" supplied by Solvay, and "Ferlosa" supplied by Montedison, all of which are polyethylenic. Fibres of other polyolefins may be used.

Although synthetic woodpulp fibres produce reasonably strong paper webs when blended with cellulosic fibres, it is frequently desirable to heat the web after it has been made to soften the thermoplastic material and thus to enhance the strength of the web by increasing the extent of inter- fibre bonding.

It has now surprisingly been found that the tear strength, tensile strength and stretch properties of a heat-bonded paper web made from a blend of cellulose fibres and synthetic thermoplastic fibres may be considerably enhancedby including a resinous additive in the paper web before heat bonding.

According to the invention therefore, there is provided a heat-bonded paper web comprising cellulosic fibres and synthetic thermoplastic fibres characterised in that the web also contains a resinous additive.

The resinous additive may be a synthetic or a natural material. An example of a suitable natural resin is rosin. Suitable synthetic resins include materials sold as wet- strength resins for paper, for example aminoplast resins such as melamine formaldehyde resin and urea formaldehyde resin. Melamine formaldehyde resin is particularly preferred (in this specification, the expression "resin"comprehends not only polymers having a large number of repeating units, but also so-called prepolymers or pre-condensates which have only a relatively small number of repeating units). Other materials which may be used include polyamine resins, such as epichlorohydrin-modified polyamine or polyamidepolyamine resins, polyethylene imine resins, and the resins sold as "Kymene" by Hercules Powder Company and "Nopcobond" by Diamond Shamrock Corporation.

The amount of resjnous additive to be used is of the order of a few per cent, based on the total weight of the paper. Above a certain % addition, the improvement in properties after heat bonding levels off. For melamine formaldehyde resin, optimum results art achieved with additions of at least 2%.

The relative proportions of cellulosic and synthetic thermoplastic fibres in the web may vary widely. Enhanced properties are obtained for example at 25%, 50% and 75% synthetic contents. Preferably however, the amount of synthetic fibres is from about 30% to about 50% based on the total fibre content. The type of cellulosic pulp used is not critical.. Bleached or unbleached softwood or hardwood kraft pulps may for example be used.

In the case of a cross-linkable resin, such as a cross-linkable melamine-formaldehyde resin, a pre-heating step may be carried out to cure the resin before heat bonding at a higher temperature is carried out.

The resinous additive may be incorporated in the web by methods normally used in the paper industry for the inclusion of additives. Beater addition is preferred.

The furnish should be relatively free-beaten if it is desired to achieve an especially stretchable product.

Heat bonding may be carried out by conventional techniques such as passage round a heated roller or passage through a heating tunnel.

The present invention is applicable to the manufacture of products for a range of uses, but is particularly suited to the manufacture of base paper for bookbinding. Such paper needs to have good tear strength and tensile strength, and to be capable of stretching to a considerable degree. It is also desirable that it should be capable of easily accepting an emboss, for example a simulated leather emboss. Such papers are conventionally made from latex containing wholly cellulosic webs. The present invention thus makes it possible to dispense with the need to incorporate latex into the paper-making furnish or with the need for a separate saturation step.

The invention will now be illustrated by the following examples, in which all percentages are by weight, and the synthetic fibres in every case were polyolefin fibres:-

### EXAMPLE 1

Four sets of laboratory handsheets of substance 100 g/m ² were prepared using a 50% woodpulp - 50% synthetic furnish (the woodpulp was a bleached softwood kraft pulp). One set contained no additives, the second a 2% Kymene resin addition, the third a 2% melamine formaldehyde addition, and the fourth a 2% rosin addition. The melamine formaldehyde and rosin additions were made in the presence of alum. The tear strength, tensile strength and stretch properties were then determined. The sheets were then heat-bonded in a laboratory oven for a period of 3 minutes at a temperature of 160°C. The tear strength, tensile strength and % stretch properties were then re-measured. The mean results are set out in Table 1 below:-

It will he seen that in each case, the properties obtained with resinous additives in the sheet are considerably better than those obtained in the absence of additives.

### EXAMPLE 2

This demonstrates the effect of different levels of melamine formaldehyde addition. 100 g/m² handsheets were made by the procedure generally described in Example 1, and the results obtained are set out in Table 2 below:-

It will be seen that whilst a 3% melamine formaldehyde addition produces the most significant enhancement in the properties measured, above 2% addition there is little further effect.

### EXAMPLE 3

This demonstrates that the melamine formaldehyde additive may be pre-heated to cure the resin before heat bonding treatment is carried out. The procedure involved taking some of the 2% MF handsheets prepared for Example 2 above and stoving them in an oven at 105°C for ten minutes before carrying out the three minute heat-treatment at 160°C.

The results obtained were as follows:-

It will be seen that although these results are marginally worse than obtained with a 2% MF addition without stoving, they represent a significant improvement on the values obtained without any additive.

### EXAMPLE 4

This illustrates the effect of changing the relative proportions of cellulosic and synthetic fibres in the sheet. 100 g/m² handsheets containing 3% MF were prepared from furnishes containing 75%, 50%, 25% and 0% synthetic fibres. The sheets were heat bonded in a laboratory oven at 160°C for 3 minutes, and the tear strength, tensile strength and % stretch properties were measured. The results for the bonded sheets are as shown in Table 4 below:-

It will be seen that the greatest improvement in properties occurred with a 50% synthetic content.

## Claims

1. A heat-bonded paper web comprising cellulosic fibres and synthetic thermoplastic fibres characterised in that the web also contains a resinous additive.

2. Paper as claimed in claim 1, characterised in that the synthetic thermoplastic fibres are present in an amount of from 30 to 50% of the total fibre content.

3. Paper as claimed in claim 1 or 2, characterised in that the resinous additive is rosin.

4. Paper as claimed in claim 1 or 2, characterised in that the resinous additive is a wet strength resin.

5. Paper as claimed in claim 1 or 2, characterised in that the resinous additive is a polyamine resin.

6. Paper as claimed in claim 1 or 2, characterised in that the resinous additive is a polyamide-polyamine resin.

7. Paper as claimed in claim 1 or 2, characterised in that the resinous additive is a polyethylene-imine resin.

8. Paper as claimed in claim 1 or 2, characterised in that the resinous additive is an aminoplast resin.

9. Paper as claimed in claim 8, characterised in that the aminoplast resin is a melamine-formaldehyde resin.

10. Paper as claimed in claim 9, characterised in that the melamine-formaldehyde resin is present in an amount of at least 2% of the total weight of the paper.
